

April 14, 1931.

T. LEWIN

1,800,457

PROCESS FOR THE REGENERATIVE TREATMENT OF ELECTROLYTE

Filed Sept. 9, 1927



INVENTOR  
Tannie Lewin

By George Lewin  
ATTORNEY

## UNITED STATES PATENT OFFICE

TANNIE LEWIN, OF UNIVERSITY CITY, MISSOURI

## PROCESS FOR THE REGENERATIVE TREATMENT OF ELECTROLYTE

Application filed September 9, 1927. Serial No. 218,491.

This invention relates to certain new and useful process for the regenerative treatment of electrolyte.

Under date of February 23, 1926, United States Letters Patent No. 1,574,043 were granted me for process for the separation and recovery of the copper, tin, and lead content of brass or bronze secondary metals or their residues. Reference is here made 5 to such Letters Patent for a full and complete disclosure and description of said process, which I will herein descriptively designate as the main process. Suffice it now, for present purposes, to state that, as steps in 10 said main process, the metals or their residues under treatment are cast into forms adapted for use, and then utilized, as anodes in an electrolytic bath in suitable electrolytic tanks, where, by the process of electrolysis, (1) the 15 copper content of such anodes is electrolytically extracted and deposited upon the cathodes, and (2) the tin and lead content or values of such anodes are, through dissolution or disintegration, removed or separated 20 out and deposited and precipitated as slime upon the bottom of the electrolytic cells.

The electrolyte employed in practicing said process is of standard composition, comprising, as its ingredients, as is usual, copper, sulphuric acid, and water in such relative proportions to accomplish and effect the best 25 results.

The actions and results obtained in practicing and carrying on said main process, 30 however, necessarily injuriously or deleteriously affect the strength of the electrolyte for continued use, and it hence becomes necessary, for the successful operation on a commercial scale of my main process, that the 35 electrolyte be regeneratively treated specifically for (1) the removal of the tin and antimony that accumulate therein from the anodes; (2) the replenishment of its sulphuric acid content, consumed by the lead, tin, and 40 other ingredients from such anodes; and (3) the replenishment also of its copper content, depleted by the cathodes due to the relatively low copper content of the anodes.

My present invention, therefore, has for 45 its object, and resides in, the provision of an

auxiliary or supplemental process whereby the electrolyte may be regeneratively treated, efficiently and economically, for continued use in the carrying on, on a successful commercial scale, of my said main process.

To such end and in the present regenerative treatment of the electrolyte, as illustrated in the accompanying diagrammatic or so-called flow drawing, used electrolyte, that is to say, electrolyte previously employed in practicing 55 or in the carrying on of the main process, is permitted to flow or circulate from the electrolytic cells A into a tank or other suitable receptacle B, where such electrolyte is subjected to heat and its temperature thereby 60 raised to a temperature varying between, say, 150° F. and boiling point (212° F.). Such heating effectively facilitates precipitation of the contained tin and antimony as basic sulphate, and I might here state that while a 65 certain amount of hydrolysis will take place without heating the electrolyte, the precipitation is soon halted on attainment of the hydrolytic equilibria of the reacting substances, when hydrolysis stops and equilibrium sets in. On the other hand, the hydrolysis of the salts is accelerated and the degree 70 of hydrolysis increases as the temperature rises, the most rapid reaction or precipitation occurring, as I have discovered, when the electrolyte is heated to a temperature of between 185° and 200° F., precipitation taking place 75 more slowly as the temperature of the electrolyte decreases to 150° F., at which latter temperature precipitation is very slow.

I then add from a tank C to the electrolyte a suitable and required amount of sulphuric acid, the quantity of which is commensurate with the former and original sulphuric acid content of the electrolyte and 80 may vary according to the nature and composition of the anodes being treated in practicing my main process.

The temperature of the electrolyte, with its sulphuric acid content restored as described, is maintained to between 130° and 212° F., and from tank B electrolyte is then 85 passed and circulated through a tank or container D for the addition to the electrolyte 90 of a proper amount or proportion of copper 100

sulphate crystals. Tank D is accordingly suitably provided and equipped with a copper mass E in the form preferably of granules, sheet copper, copper borings, copper turnings, copper clippings, copper wire, copper mill scale, copper sludge, or the like, presenting relatively large surfaces for air contact. Such passing and circulating of so partially restored electrolyte through the copper mass is preferably with air contact, and for such purpose I might here state that, to most effectively obtain proper air contact while electrolyte is circulating through the copper mass, the electrolyte is preferably sprayed intermittently, as by means of a suitable pump or other spraying device, F, G, from tank B over and through the copper mass E in tank D, the intermittent spraying being so regulated as to allow and permit sufficient time for the air to come in contact with the copper mass, and the so treated electrolyte then circulating through a line or pipe H to a suitable supply-tank J, from whence the regenerated electrolyte again passes or circulates into the electrolytic cells A.

To obviate the addition to the electrolyte being treated of a content of copper sulphate crystals excessive for practicing the particular process of electrolysis to be carried on, preferably but a regulated or controlled part of the electrolyte under treatment is sprayed and circulated through tank D. Hence, the tank B also preferably communicates through pump F and by means of a line or pipe K with the supply-tank J, with which pipe or line K the tank D has valve-controlled communication as by means of a by-pass L.

In such manner, the electrolyte being at the proper temperature, I effect the addition and restoration to the electrolyte of copper sulphate crystals in such amount or quantity to replenish substantially the former and original copper content of the electrolyte for effectively practicing and carrying on my main process.

The regenerated and restored electrolyte is then, as I have stated, passed through from tank J to the electrolytic cells A for re-use in practicing and carrying on my main process.

I am aware that changes in the several steps of my process may be made and substituted for those herein described without departing from the nature and spirit of my invention.

Having thus described my invention, what I claim and desire to secure by Letters Patent is:

That step in the process of purifying and regeneratively treating used electrolyte for employment in the electrolytic removal from brass or bronze secondary metals or their residues of their copper, tin, and lead content, which consists in heating the electrolyte after removal from the electrolytic cell to a

temperature between 150° F. and 212° F. for accelerating the rate of hydrolysis of its tin and antimony content.

In testimony whereof, I have signed my name to this specification.

TANNIE LEWIN.

70

75

80

85

90

95

100

105

110

115

120

125

130